

June 4, 1957

C. A. TURNER, JR

2,794,630

APPARATUS FOR HEAT TREATING STRIP MATERIAL

Filed Dec. 12, 1951

FIG. 1



FIG. 2



INVENTOR.  
CHARLES A. TURNER JR.

BY *J. W. Sorenson*

ATTORNEY.

2,794,630

## APPARATUS FOR HEAT TREATING STRIP MATERIAL

Charles A. Turner, Jr., Philadelphia, Pa., assignor to Selas Corporation of America, Philadelphia, Pa., a corporation of Pennsylvania

Application December 12, 1951, Serial No. 261,311

3 Claims. (Cl. 266—3)

The present invention relates to the continuous heat treatment of strip or strand material, and more particularly to the treatment of strip metal to place an oxide coating of a predetermined color or thickness on the surface thereof.

In continuous annealing or normalizing of strip metal as presently practiced, the aim and result is to produce bright strip which, when exposed to air immediately following the cooling under a protective atmosphere will not oxidize on its surface. Subsequently, if the strip is to be coated, it is subjected to a light pickle to remove any traces of grease or stain that might interfere with the coating process.

It has been found, however, that a very light, thin oxide film on the strip at the pickling stage would have merit in acting as the means for providing a light surface layer of reduced iron. Such a surface will provide the optimum condition for producing a tightly adherent tin-plate or galvanizing coating, for example. In such a case, the oxide film should be of a uniform color or thickness ranging from light straw to blue in appearance. Care must be exercised, however, to avoid thicker oxide films since they may have a damaging effect on the polished roll surfaces used in temper rolling which follows annealing and precedes coating. An added advantage of a tightly adherent oxide film is that it prevents atmospheric rusting or oxidation during the interval between annealing and coating, which in some cases, may be several days.

It is an object of the invention to provide a method and apparatus for placing an oxide film of controlled thickness upon the surface of a metal strip or strand.

It is a further object of the invention to provide a method and apparatus for placing an oxide film of controlled thickness upon the surface of a continuously moving metal strip. Such method and apparatus is preferably used in combination with a continuous strip annealing or normalizing apparatus.

In carrying out the invention, strip is heated and cooled in a conventional strip annealing or normalizing apparatus that is designed to produce a bright strip. The strip is removed from said apparatus at a temperature at which it will oxidize in air, and is kept in an oxidizing atmosphere for the time required for the strip to obtain an oxide film of the desired thickness. Thereafter, the strip is quenched to a temperature below that at which it will oxidize in the air. The color or thickness of oxide coating obtained will vary with the time the strip is exposed to said atmosphere. This time may be varied either by moving the strip varying distances at a given speed before it is quenched, or by moving it a given distance at varying speeds before quenching.

In the description, the material being treated is referred to as a strip. It should be understood, however, that the material can be in strand or other form adapted for continuous treatment. While the apparatus is particularly designed for the treatment of tin-plate stock such as cold rolled, low carbon strip, it will be understood that it

may be used with any material for which the treatment is beneficial or desired.

The various features of novelty which characterize my invention are pointed out with particularity in the claims annexed to and forming a part of this specification. For a better understanding of the invention, however, its advantages and specific objects attained with its use, reference should be had to the accompanying drawings and descriptive matter in which I have illustrated and described a preferred embodiment of the invention.

In the drawings:

Figure 1 is a diagrammatic view, partly in section, of the apparatus for carrying out the invention, and

Figure 2 is a view in section showing a modified form of the invention.

Referring to Figure 1, the strip S is brought in from the left of the drawing from some suitable source of supply and is passed over a guide roller 1. From here, it moves vertically downward through a furnace 2 having in it a furnace chamber 3. This furnace serves to heat the strip to an annealing or normalizing temperature in the range of 1200° F. to 1700° F. From the furnace, the strip passes through a suitable seal 4 and into a cooling chamber 5 that is normally filled with a protective atmosphere which will insure that the surface of the strip is bright when it leaves the chamber. The cooling chamber is provided with a series of guide rollers 6 over which the strip travels in a series of loops while it is being cooled from the temperature to which it was heated in the furnace to a temperature below which the desired metallurgical changes have occurred, but above a temperature at which it will oxidize in the atmosphere. Preferably, however, the temperature will be in the range of from 450° F. to 900° F. It is noted that partitions 7 may be placed in the cooling chamber between each of the convolutions of the strip in order that the cooling thereof may be controlled more closely than would otherwise be the case.

The strip leaves the cooling chamber through a suitable roll seal 8, that serves to prevent the entrance of air to the cooling chamber, and passes around a pair of guide rollers 9 and 10 that are located in a quench tank 11. Upon leaving the quench tank, the strip goes over a guide roller 12 and through pinch rollers 13. These rollers serve to move the strip through the heating and cooling chambers as well as through the quench tank. They are driven by a motor 14 whose speed may be controlled with a conventional controller 15. The cooling tank is provided with a partition 16 which serves to divide it into an entrance portion that is supplied with a quench fluid, such as water, through a pipe 17 at a rate that is controlled by a valve 18 in the pipe. The quench fluid flows from the tank through an outlet 19 having a swivel joint 20 therein, and an adjustable pipe 21 into a drain 22. The angle of the pipe 21 may be adjusted, thereby adjusting the level of the liquid in the quench tank. To this end, pipe 21 is provided with a yoke 23 that has pivoted to it a threaded shaft 24. This shaft passes through a frame 26 and receives thereon a hand wheel 25. The angle of the pipe 21 can be adjusted, thereby varying the level of the liquid in the tank, by the rotation of hand wheel 25.

In the operation of this system, strip is fed into the heating chamber continuously and at a speed that is regulated by the adjustment of motor 14. This speed is such that in conjunction with the firing of the furnace, the temperature of the strip is raised to 1200° F. to 1700° F. during its passage through the furnace chamber 3 depending upon whether it is being annealed or normalized. Upon leaving the furnace, the strip passes through the seal 4 and into the cooling chamber 5. A

protective atmosphere is maintained in this chamber so that the strip will be kept bright while it is cooling. In other words, the heating and cooling chambers actually heat treat the strip and deliver a bright strip through the roll seal 8 into the air.

After the strip has been heated, it must be cooled at a controlled rate until its temperature has been reduced to a point where the desired metallurgical characteristics are obtained. This usually occurs by the time the strip has reached 900° F. Any cooling beyond a small amount below this point is ordinarily undesirable because of the expense and the mechanical difficulties that are encountered. In order to carry out the present invention, however, it is only necessary that the strip be above a temperature at which it will readily oxidize in air. This is about 450° F. Therefore, the cooling effect of the cooling chamber is adjusted by conventional means so that the strip is discharged into the air at any temperature in the range of 450° F. to 900° F., but preferably between 750° F. and 800° F. At this temperature, the amount of oxidation will depend upon the time of exposure. Therefore, at a given speed of the strip, a predetermined color or thickness of oxide coating will be placed upon its surface, depending upon the length of time required for the strip to move from the roll seal 8 into the quench liquid in tank 11. By varying the level of the liquid in the tank, the distance that the strip travels and the time that the strip is exposed to the air will be varied, and therefore, the color of the oxide film placed on the strip will be varied.

It has been found in a number of cases, particularly where the strip is later to be used for tin-plating or galvanizing, that it is advantageous to have a thin oxide film on the surface of the strip. When the strip is subjected to a pickle prior to the coating, reduction of the oxide film by the pickle bath will leave a microscopically thin layer of sponge iron on the surface to which the coating seems to adhere more tightly than if the layer were not there. The thickness of the layer of sponge iron can be varied by the thickness of the oxide coating placed on the strip surface. Generally this will be from light straw to blue. Such a coating can be placed on the surface of the strip in a few seconds, so that the distance the strip travels in the air after it leaves the cooling chamber and before entering the quench tank can be relatively short.

Alternately, the level of the liquid in the quench tank can be maintained constant, and the thickness of the coating on the strip can be varied by varying the speed thereof. In either case, the result is the same. The thickness of the oxide film placed on the surface of the strip is strictly a function of time and temperature. If the strip is at a given temperature, the oxide film will be placed on its surface in a given time. The annealing apparatus is so adjusted that the exit temperature of the strip can be predetermined. Therefore, the thickness of the oxide film is varied by either changing the speed of the strip or by varying the level of the quench liquid since both of these determine the time that the strip is traveling in the air.

The temperature of the quench fluid, ordinarily water, can be maintained at any desired value just so that the strip, when it leaves the quench tank, is below a temperature at which it will oxidize in the air. Normally, it is desirable to keep the temperature of the water at approximately 180° F. When this is the case, the strip can be dried in the air due to evaporation of the water from it with a minimum of trouble. When the liquid is cooler, say at room temperature, provisions must be made for blowing hot air over the strip in order to dry it before it is coiled to be stored until use. The temperature of the quench water can be controlled by varying the volume of water that passes through the quench tank. The arrangement of the tank is such that water is introduced into a compartment which is separated from the main

part of the tank thereby reducing turbulence of the water. This insures that the level of the water can be maintained accurately. The arrangement is also such that the heated water is removed from a point adjacent to the entrance of the hot strip. This makes it easier to keep the temperature of the water at the desired value than would be the case if the water was withdrawn from the tank at some point remote from that at which the strip entered.

At times, it may be difficult to obtain an even oxide coating on both sides of the strip due to various plant conditions. If there is a draft blowing in one direction, for example, the strip may be oxidized more on one side than on the other side. For this reason, it may be desirable to protect the strip between the roll seal 8 and the quench liquid. If such a construction is necessary, there can be provided a shield 27, as indicated in Figure 2. This shield will extend from the rolls downwardly to a point beyond the lowest level that the water in the quench tank will reach. The supply of oxygen in the shield will soon be exhausted unless a continuous supply thereof is provided. To this end, an inlet pipe 28 extends into each side of the shield through which air or oxygen enriched air may be introduced. The inner end of each pipe terminates in a discharge outlet 29 which outlets are so arranged that the air blown through them will impinge against the side walls of the shield and be diffused evenly through the area thereof. In view of the fact that the strip is heated, it will raise the temperature of the quench liquid above the boiling point so that the shield eventually will become filled with steam unless provision is made to remove it. For this reason, there is provided an outlet 31 through which the steam can be removed from the shield. This outlet will have to be above the level of the quench water at its highest point. If desired, the outlet could be arranged to move upwardly and downwardly with the level of the quench liquid so that it is just above the liquid level. In this manner, steam can be withdrawn from the shield at the point where it is formed.

As was mentioned above, the atmosphere in the cooling chamber 5 is a protective atmosphere that will deliver a bright strip through the roll seal. If air, or oxygen enriched air is introduced at a high pressure into the sleeve 27, there will be a tendency for this air to flow upwardly through the roll seal 8 into the cooling chamber. Such a procedure is undesirable, since the effect of the protective atmosphere in the cooling chamber would be ruined. Therefore it is necessary by the use of any conventional pressure control apparatus to maintain in the sleeve 27 a pressure which is slightly lower than the pressure which is maintained in the cooling chamber 5. In practice, air or other oxidizing gas is continuously introduced through inlets 28 and exhausted along with the steam through outlets 31. The slight circulation of air in the sleeve 27 insures that there will be at all times an oxidizing atmosphere which is sufficient to place an oxide coating on the surface of the strip.

Whether the strip is open to the air as shown in Figure 1, or is in a protective sleeve as is shown in Figure 2, the result and operation of the system is the same. In each case, the hot strip is moved through an oxidizing atmosphere for a time sufficient for an oxide coating of desired color to be placed on its surface. Whether or not the shield is used will depend mainly upon the conditions in a particular plant.

From the above description, it will be seen that I have provided a method and apparatus for placing an oxide film of predetermined thickness upon the surface of a strip of material. The process and apparatus are particularly adapted for use in connection with the annealing of cold rolled, low carbon steel of the type that is generally used for tin-plate. It will be apparent, however, that the apparatus can be used in connection with any material upon which it is desired to place an oxide film.

It is also useful in connection with strands or wires as well as with strip material.

While in accordance with the provisions of the statutes, I have illustrated and described the best form of embodiment of my invention now known to me it will be apparent to those skilled in the art that changes may be made in the form of the apparatus disclosed without departing from the spirit and scope of the invention, as set forth in the appended claims, and that in some cases certain features of my invention may be used to advantage without a corresponding use of other features.

What is claimed is:

1. Apparatus for heat treating a metal strip comprising in combination means to deliver bright strip metal at a temperature in the range of 450° F., to 900° F., an open quench tank located directly in line with the delivery end of said means, guide rollers to guide the strip through said quench tank, means to direct an oxidizing atmosphere against the strip as it moves between said means to deliver and through said quench tank, means to move the strip from said means to deliver and through said quench tank at a constant speed, means to vary the level of a quenching fluid in said quench tank to thereby vary the time required for the strip to travel through said oxidizing atmosphere from said means to deliver until it is immersed in the quenching fluid said means to direct including a duct through which the strip travels between said means to deliver and said quench tank, and means to introduce an atmosphere having an oxidizing effect into said duct. 25

2. Apparatus for placing an oxide coating on the surface of a strip of metal comprising in combination mechanism to bright anneal continuously a strip of metal and having a delivery opening through which said strip is discharged in a downward direction into the air, said mechanism having means to deliver strip therefrom at a temperature above which it will oxidize in air, quench

means located immediately below the delivery opening of said mechanism, the strip traveling through air between the delivery opening and said quench means, drive means to move said strip at a constant speed, and means to vary the height of said quench means relative to said delivery opening to thereby vary the time said strip is exposed to the air.

3. Apparatus for heat treating a metal strip comprising in combination mechanism to heat and cool a strip, 10 said mechanism including means to discharge said strip at a temperature above which it will oxidize in air, a quench tank, guide means to guide said strip directly from said discharge means to and through said tank, means to move said strip through said mechanism and said tank, adjustable means to maintain various predetermined levels of a quenching fluid in said tank, a shield surrounding said strip and extending from said discharge means to a point below any level of the quenching fluid in said tank, and means to supply an atmosphere having 15 an oxidizing effect on said strip into said shield. 20

#### References Cited in the file of this patent

#### UNITED STATES PATENTS

|    |           |               |               |
|----|-----------|---------------|---------------|
| 25 | 627,022   | Theobald      | June 13, 1899 |
|    | 854,810   | Daniels       | May 28, 1907  |
|    | 1,362,213 | Andrews       | Dec. 14, 1920 |
|    | 1,704,015 | Naugle et al. | Mar. 5, 1929  |
|    | 2,110,893 | Sendzimir     | Mar. 15, 1938 |
| 30 | 2,137,817 | Tuerff        | Nov. 28, 1938 |
|    | 2,283,109 | Von Ende      | May 12, 1942  |
|    | 2,340,461 | Gage et al.   | Feb. 1, 1944  |
|    | 2,418,087 | Nachtman      | Mar. 25, 1947 |
|    | 2,420,377 | Jones         | May 13, 1947  |
|    | 2,546,538 | Erhardt, Jr.  | Mar. 27, 1951 |
|    | 2,594,876 | Cope          | Apr. 29, 1952 |